

C. H. Brady,

*Casting Plow-Shares.*

N<sup>o</sup> 35,744.

*Patented July 1, 1862.*



Witnessed  
and stamped  
H. B. McNeal

Inventor:  
Christ. H. Brady

# UNITED STATES PATENT OFFICE.

CHRISTIAN H. BRADY, OF MOUNT JOY, PENNSYLVANIA.

## IMPROVEMENT IN MOLDS FOR CASTING PLOWSHARES.

Specification forming part of Letters Patent No. 35,744, dated July 1, 1862.

*To all whom it may concern:*

Be it known that I, CHRISTIAN H. BRADY, of Mount Joy, in the county of Lancaster and State of Pennsylvania, have invented a new and Improved Flask and Mode of Casting and Chilling Plow-Irons in a Vertical Position; and I do hereby declare that the following is a full and exact description thereof, reference being had to the accompanying drawings, and to the letters of reference marked thereon.

Figure 1 is a perspective view of the flask with the pattern *c* within ready for molding. Fig. 2 represents the two faces of the pattern or mold-board used in this illustration. Fig. 3 is the chill-drag or nowel forming the side *B* of the flask, Fig. 1. Fig. 4 is the cope, (marked *A*) shown detached, all made of cast-iron.

To enable others skilled in the art of casting to use my invention, I will more fully explain the features I deem new and peculiar in the mode and flask employed.

My chill-drag or nowel *B*, Fig. 3, consists of a smooth casting having the face curved and shaped for the reception of the pattern of the mold-board to be cast. This drag has a broad flanged edge, *F*, with three snugs or ears, *E*<sup>2</sup>, which are perforated to receive the pins on the ears *E'* of the cope *A*. There is also a box with beveled sides *K*, for molding the head *H* of *C*, 1 and 2. This box has a series of perforations in its bottom, and forms one-half of the runner *M*. There are also perforations *G* inside the flange *F* for the escape of gases generated while casting or filling in. This drag has also lugs *L L L* on its face, in order to form the holes *P P P* in the pattern, or, rather, castings taken therefrom. The cope *A*, Fig. 4, with its lugs *E'*, handles *R*, and curved cross-pieces 1, 2, and 3, is also cast and corresponds in shape and curvings, so as to adapt it at all points to the drag and pattern, which unite and lock, forming the flask, Fig. 1.

Sand is put in the box *K*, and the pattern is laid on the smooth face of the cast nowel, the cope put in place and well packed with sand in the ordinary way. When properly molded, the pattern is removed and the flask secured in a vertical position. The usual precaution may be employed to prevent the mold from giving way while casting, by the application of a flat board or plate against the cope, the beveled sides of which are deemed a sufficient protection, however. The metal is poured in through the runner *M*, formed on the top of the flask by the union of the nowel and cope *B A*. The smoothness and hardness of plows are highly important, and to gain this object, so much needed and partially attained by chilling mold-boards cast in the ordinary wooden flasks in a horizontal position, they are by this improved flask chilled while cast in a vertical position, thereby making the most perfect castings, of a polish and hardness so vastly superior to any cast in the ordinary way as to constitute the device employed as novel as the result, which latter is of the greatest utility and deemed a highly important improvement. Thus I admit that I am aware that chilling plow-irons is not new in the ordinary horizontal position.

I am also aware that cylinders, and perhaps other castings, have been cast in a vertical position; nor do I claim the mere chilling and vertical casting separately considered.

What I claim as my invention, and desire to secure by Letters Patent, is—

1. The combination of the flask formed by the chill-drag or nowel *B* and cope *C*, arranged substantially in the manner set forth.
2. Casting and chilling plow-irons in a vertical position by means of such a flask.

CHRIST. H. BRADY.

Witnesses:

JACOB STAUFFER,  
H. B. McNEAL.